

# UNITED STATES PATENT OFFICE.

GILBERT E. BAILEY, OF LOS ANGELES, CALIFORNIA, ASSIGNOR TO FERROCHEM COMPANY, A CORPORATION OF ARIZONA.

## COMPOSITION FOR TREATING BOILER FEED-WATER.

1,096,344.

Specification of Letters Patent. Patented May 12, 1914.

No Drawing. Original application filed November 28, 1910, Serial No. 594,585. Divided and this application filed August 4, 1913. Serial No. 782,961.

To all whom it may concern:

Be it known that I, GILBERT E. BAILEY, a citizen of the United States, residing at Los Angeles, in the county of Los Angeles and State of California, have invented a new and useful Composition for Treating Boiler Feed-Water, of which the following is a specification.

My invention is a composition of matter which I introduce into the feed water entering a steam boiler and the objects of my invention are, first, to provide a composition that will prevent the formation of scale upon the evaporative surfaces of such a boiler; second, to provide a composition that will neutralize certain of the impurities contained in such boiler feed water and prevent them from attacking the shell or other metal parts of such a boiler; and third, to provide a composition that will prevent the said shell from being disintegrated by electrolytic action.

My composition consists of a mixture of graphitic iron with from one to four per cent. of zinc and this composition is that disclosed in my application for a United States patent on alloy and process of making, Serial 594,585, filed November 28, 1910, of which this is a division.

It is adapted to be used in the place of the expensive and bulky chemicals generally known as boiler compounds and it may be used in the form of a dust or powder, or lathe turnings, added direct to the water in the boilers. It may be cast into machines or mechanical devices in which the boiler feed water is brought into intimate contact with it, whereby the mineral matter in solution is acted upon to accomplish the above objects. In practice I prefer to introduce the composition into the feed water by reducing it to small particles by abrasion. Such small particles may be introduced into the water by several different methods such as first, by providing a composition composed of graphitic iron and zinc, and providing means for feeding particles of this composition to the water. Second, by producing an alloy of graphitic iron and zinc and thereafter providing an abrasion whereby particles of said alloy are fed into the feed water.

The processes whereby the compositions used in the first method given above are produced are evident consisting simply of ordinary

grinding or other methods of dividing the constituent materials, and a suitable mixing in the proper proportions.

The process of producing the composition used in the second method given above has been fully disclosed in my application, Serial 594,585, of which this is a division. In the composition used in this second method the iron is present as an iron reasonably free from such impurities as sulfur, phosphorus, silicon and the like, and the iron is not united in chemical combination with the carbon. The carbon is largely or wholly free and in the form of graphite the mixture being what is usually called graphitic iron. The zinc is a mixture or alloy with the iron and not a chemical combination. The composition is soft, flaky and friable under rubbing or abrasive action.

The composition used in the second method given above is made as follows: A pig iron is selected that is as free as possible from impurities and that carries as high a percentage of carbon as possible. Imported Chinese pig iron and the Scotch pig irons, rich in carbon, answer the purpose. The pig iron is melted in any foundry stack furnaces using such fluxes as any one skilled in the art of refining iron would use, the main object being to produce an iron free as possible from sulfur, arsenic, silicon, and other impurities, and yet keep the carbon contents high. When the iron is tapped from the furnace into the pouring ladle, from one to four per cent. of pure metallic zinc is added according to the way the metal will be finally used. In castings one or two per cent. of zinc is found to work well. If the composition is to be made into powder or turned on a lathe into shavings, three or four per cent. of zinc may be added. The composition should be as hot as possible when poured. It is important that the composition should cool slowly in the mold in order to produce ferrite, and to have the carbon appear as flaky graphite. Special attention must be given to preparing the mold and cores, when cores are used. This is accomplished by the following means: Some coal tar, crude petroleum, or other oily heavy hydrocarbon is added to the molding sand so as to furnish heat to the sand and iron while the iron is cooling, without robbing the iron of any carbon. Any cores used should be made

of sand and a heavy oil such as linseed, or rape oil, and finished with a light coat of shellac. As both core and sand under this treatment give off large volumes of gas as the facing burns, it is necessary that special care be given to the vents to see that they are large, free and numerous. The composition should be left in the mold until cold enough to handle with the hands, or left at least two hours after pouring before taking out of the mold. The cast composition should under no circumstances be cooled rapidly or have water thrown upon it, as, to do so, produces cementite and defeats to that extent the purpose of the composition.

I have found that the methods and compositions disclosed above are quite efficient in accomplishing the objects previously stated herein.

I believe that to produce a successful boiler feed water purifier all of these objects should be accomplished and I further believe that each of the elements of my composition contributes to the successful accomplishment of each object. I further believe that the

accomplishment of these objects, particularly the second, is in part at least dependent upon certain mechanical actions in the boiler such as a colloidal or similar action which prevents the foreign matter from cementing to form scale. I prefer, however, not to discuss the theory involved in the action of my invention contenting myself with a disclosure of the manner of making and using same in such full, clear, concise and exact terms as to enable any person skilled in the art to which it pertains to make, construct, compound and use the same.

I claim as my invention:

A composition containing substantially 40 pure iron, carbon in the form of graphite and from one to four per cent. of zinc.

In testimony whereof, I have hereunto set my hand at Los Angeles, California, this 26th day of July, 1913.

GILBERT E. BAILEY.

In presence of—

FRED A. MANSFIELD,  
FORD W. HARRIS.